

Aug. 3, 1937.

H. H. HARRIS

2,088,593

CARBURIZING BOX WITH INNER SURFACE RESISTANT TO CARBON PENETRATION

Filed May 1, 1935.



INVENTOR  
HENRY H. HARRIS.

BY  
Dyke and Schaines

ATTORNEYS

## UNITED STATES PATENT OFFICE

2,088,593

CARBURIZING BOX WITH INNER SURFACE  
RESISTANT TO CARBON PENETRATION

Henry H. Harris, Boston, Mass.

Application May 1, 1935, Serial No. 19,196

2 Claims. (Cl. 263—49)

My invention relates to carburizing boxes and has for its object to provide a carburizing box which is made of reduced porosity and increased 5 resistance to carbon penetration by coating the interior with a suitable material such as nickel, copper or the like.

In the drawing annexed hereto, and made a part hereof:

Figure 1 is a perspective showing a conventional carburizing box undergoing the treatment of 10 my invention, the details being exaggerated for illustrative purposes; and

Fig. 2 is an enlarged similarly exaggerated sectional view through one wall thereof on the line 15 2—2.

The carburizing box 10 is made of suitable material, such as nickel-chromium-iron alloy, and by my invention same can be of relatively lower alloying constituents, such as lower nickel 20 and chromium by reason of the provision of the interior coating of nickel, etc., as stated, thereby obtaining equal life with lower expense for alloying constituents, or increased life for the same expense put into alloying constituents.

The interior coating 12 may be applied in various ways but it is preferably applied by spraying with the well known Shoup gun 14 whereby the coating material is sprayed as it is melted.

While not always essential, the deposited metal 30 is preferably swedged to close up its surface grain and give it a smoother and better surface and to force the coating into any small depressions or irregularities in the original interior surface of the box.

A single coating is ordinarily sufficient, but plural applications may be made if desired, preferably with swedging after each application.

Nickel gives the best results when applied with the Shoup gun to the interior carburizing boxes of nickel and chromium alloy constituents, serving effectually to close the pores and to give added resistance to carbon penetration, but materials such as copper and the like may be used to substantial advantage.

The materials used are preferably those having considerable pliability, ductility and toughness, and which are not greatly different in coefficient of expansion from the alloy material to which the coating is applied so that parting and spalling are avoided in use under the high temperatures and severe conditions to which exposed, nickel and copper being well adapted in those respects. When the box alloy material comprises nickel, a metallic coating also comprising nickel is well 20 adapted for the purposes of my invention.

I claim:

1. A carburizing box of alloy material comprising nickel, chromium, iron, etc., having a spray deposited interior surface layer of nickel.

2. The process of imparting enhanced chemical and physical resistance to carbon penetration to a carburizing box of an alloy material comprising nickel, chromium, iron, etc., which consists of spraying the interior surface of the box with nickel in molten, finely-divided state, thereby depositing a layer of nickel thereon.

HENRY H. HARRIS.